

Patented May 15, 1951

2,553,396

# UNITED STATES PATENT OFFICE

2,553,396

## ROSIN AMINE TREATED NATURAL CELLULOSE FIBERS

Joseph M. Almand, Hogansville, Ga., assignor to  
United States Rubber Company, New York,  
N. Y., a corporation of New Jersey

No Drawing. Application August 2, 1948,  
Serial No. 42,140

15 Claims. (Cl. 8—116.2)

1

This invention relates to improved cellulosic fibers, yarn or cord and a method of improving its tensile strength.

U. S. patent to H. M. Buckwalter No. 2,297,536 covers the treatment of native cellulosic fibers with non-volatile, non-waxy, water-soluble, cotton-wax-peptizing agents which contain a tricyclic hydroaromatic condensed nucleus, particularly with aqueous solutions of alkali metal salts of rosin acids and their derivatives to improve the tensile strength thereof. U. S. Patent 2,422,078 to the same inventor similarly covers the treatment of native cellulosic fibers with aqueous solutions of alkali metal salts of acids of "run" native Congo copal resin. One of the results brought about by the treatments covered in these patents is a substantial and commercially important increase in the tensile strength of the cotton yarns, cords, etc. The treating agents mentioned may be referred to as being active and the degree of activity which they possess may be expressed in terms of the percentage increase in tensile strength which they impart to grey cotton fiber.

I have now found that condensed and uncondensed polynuclear hydroaromatic primary amines possess textile strength-improving activities comparable with those exhibited by the treating agents referred to above, particularly the alkali metal salts of the rosin acids. The amine may be used either as such or in form of a salt thereof. Where the amine itself is used, I prefer to apply it to the grey cotton yarn or the like in the form of an aqueous dispersion thereof or in the form of an aqueous emulsion of a solution of the amine in a suitable volatile organic solvent. The amine could also be applied in the form of a solution in a volatile organic solvent.

I prefer however to apply the amine in the form of a water-soluble salt thereof in solution in water.

Any polynuclear hydroaromatic primary amine may be used in the practice of my invention. An example of an uncondensed polynuclear hydroaromatic amine which can be used in the present invention is orthoaminodicyclohexyl. I prefer, however, to employ the amines which contain a condensed tricyclic hydroaromatic nucleus and particularly such amines which have the general formula



2

where ring A is a hydroaromatic ring, where ring B may be hydroaromatic or semi-aromatic and where ring C may be hydroaromatic, semi-aromatic or aromatic. Specific examples of such condensed polynuclear hydroaromatic amines are dehydroabietylamine, tetrahydroabietylamine, dihydroabietylamine and dextropimarylamine, and particularly a mixture of the latter four amines which is known commercially as "Rosin Amine D" which is described by J. N. Borglin in an article appearing in "Soap and Sanitary Chemicals," December 1947. The major components of "Rosin Amine D" are stated by Borglin to be as follows:

15



20



25



30



35

40

The components of "Rosin Amine D" are made from, but are not derivatives of, disproportionated rosin acids in a manner well known to those skilled in the art. Processes for effecting the disproportionation of rosin are well known in the art; processes based on the use of a palladium catalyst are described by Fleck et al., J. A. C. S., 60, 159 (1938), and by Littmann, U. S. Patent No. 2,154,629. The disproportionated rosin acids may then be converted to the corresponding primary amines in any suitable manner known to the art, for example by converting them to the nitriles and then reducing the nitriles to the primary amines. Rosin amines are described in detail in a pamphlet entitled "Rosin Amines" issued by the Naval Stores Department of Hercules Powder Company under date of February 1, 1948. "Rosin Amine D" as commercially available contains at least 88% of rosin amine and often as much as 95% thereof. A

45

50

55

60

typical analysis and characteristic physical properties of "Rosin Amine D" are as follows:

|                                              |                                 |
|----------------------------------------------|---------------------------------|
| Physical state.....                          | Viscous yellow liquid           |
| Color.....                                   | Pale yellow                     |
| Density at 25° C.....                        | 0.997                           |
| Refractive index at 20° C.....               | 1.5410                          |
| Nitrogen content.....                        | 4.2-4.5%                        |
| Bromine number (KBr-KBrO <sub>3</sub> )..... | 49                              |
| Viscosity at 25° C.....                      | 4,670 centistokes               |
| Boiling range (5 mm.).....                   | 187-211° C.                     |
| Boiling range (100 mm.).....                 | 270-291° C.                     |
| Boiling range (760 mm.).....                 | 344° C. (partial decomposition) |
| Flash point (Cleveland Open Cup).....        | 192° C.                         |
| Heat of vaporization.....                    | 20,100 calories per mole        |
| Neutralization equivalent.....               | 317                             |

Although the disproportionated rosin acids and "Rosin Amine D" have identical condensed ring structures, they differ in their respective functional groups. The functional group of the disproportionated rosin acids is —COOH (carboxyl), whereas the functional group of the compounds which are employed in accordance with the present invention is —NH<sub>2</sub> (primary amino). The water-soluble rosin acids salts are anionic (R.COO<sup>-</sup>M<sup>+</sup>) whereas the water-soluble salts of the amines used in my invention are cationic (RNH<sub>3</sub><sup>+</sup>A<sup>-</sup>) active chemicals.

Instead of dehydroabietylamine, tetrahydroabietylamine, dihydroabietylamine and dextropimarilylamine, I may use in the practice of my invention primary amines of other rosin nuclei, for example, abietylamine, dihydrodextropimarilylamine, etc. I may use in the practice of my invention the amines of the nuclei of the rosin acids found in ordinary rosin such as abietic acid, pimamic acid, sapinic acid, or in modified rosins, i. e., rosins which have been chemically modified to chemically change the rosin nucleus, e. g., heat treated rosin, isomerized rosin, polymerized rosin, hydrogenated rosin, etc. I prefer to use the mixture available commercially as "Rosin Amine D" identified above.

In the preferred practice of my invention wherein I treat the grey cotton fiber with an aqueous solution of the amine salt, I may use any water-soluble salt of the foregoing amines. The acids capable of forming sufficiently water-soluble salts of the polynuclear hydroaromatic primary amines appear to be limited to monobasic inorganic acids, e. g., hydrochloric acid, and monobasic organic aliphatic carboxylic acids having from 1 to 4 carbon atoms per molecule, examples being formic, acetic, propionic and butyric acids among the unsubstituted saturated monobasic aliphatic acids, and glycolic, lactic and alpha-hydroxy butyric acids among the alpha-hydroxy saturated monobasic aliphatic acids. Where organic acids are used to form the salt I generally use saturated acids. Attempts to make water soluble salts of such amines with inorganic and organic polybasic acids and with aromatic mono- and poly-basic carboxylic acids and with sulfonic acids have not been successful.

The hydroaromaticity of the amines used in the present invention is essential to the textile strength-improving activity of such amines. The textile strength-improving activities of aliphatic and aromatic amines are practically zero.

The amines of the present invention may be applied to the grey cotton fiber in the same manner as described in Buckwalter U. S. Patent No. 2,297,536, typically, by applying to the grey cotton yarns or the like an aqueous solution of the water-soluble salts of the amines of the pres-

ent invention followed by removal of the excess solution in any suitable manner, as by use of a vacuum, followed by drying at a suitable elevated temperature at which the water present will be driven off. The same type of apparatus as shown in that patent may be used in applying the amines of the present invention. The theory of the action of the amines of the present invention is believed to be the same as that described for the compounds covered in U. S. Patent No. 2,297,536. The treatment with the amines of the present invention confers upon the treated cotton the characteristic that it shows upon hot ethyl alcohol extraction of substantially all the alcohol-soluble material a tensile strength-improvement which can be detected but which is less than 9% and generally is less than 5%. This is in contradistinction to untreated grey cotton yarn or cord which, upon extraction of substantially all the alcohol-soluble material with hot ethyl alcohol, exhibits a gain in tensile strength of the order of 10 to 15% due to the removal of cotton waxes normally present on the fibers.

The present invention is applied to grey cotton which contains at least 75% of the original naturally occurring cotton waxes and generally substantially all of the original waxes.

Where the amine of the present invention is applied to the grey cotton yarn or the like in the form of an aqueous solution of a water-soluble salt of the amine, the concentration thereof may vary widely. However, it is preferred to employ a concentration of at least 0.5% by weight of the amine in the treating solution, concentrations below 0.5% generally giving an insufficient improvement for commercial practice. Generally speaking, above 20% concentration, the resulting solutions are too viscous for practical use. I therefore prefer to employ a concentration within the range of from 0.5 to 20%. Within this range, the improvement in tensile strength appears to increase roughly proportionally with the increase in concentration. The foregoing percentages refer to the amine as such combined in the salt rather than to the salt, although the difference is generally slight due to the high molecular weight of most of the amines used.

The invention is of special utility in connection with the production of tire cord from which rubberized fabric plies are made, which in turn become part of the pneumatic tire carcass. By reason of the improved tensile strength of the unrubberized tire cord, it is possible to make a standard quality tire with less tire cord, or in the alternative to make a superior tire with the usual quantity of tire cord. Thus the chemically treated grey cotton cords may with or without intermediate drying be immersed in a rubber latex composition for the making of weftless cord fabric for tire carcasses. The latex composition, when dry, ultimately acts to bind the cords in parallel relation.

The treated grey cotton of the present invention usually finally contains at least 0.1% by weight of the amine. The increase in weight on the bone dry basis may range from 0.1 to 2% by weight as a result of the treatment.

The invention may be applied to treating finished tire cords made of grey cotton or to grey cotton fibers in any form as for example yarn, plied yarn, cabled yarns, twisted products from plied yarns, fabrics woven from yarns or cords, unspun cotton, etc.

While rubberizing of the treated cotton has been referred to as illustrative of further processing, it will be apparent that various uses of the grey cotton will not require rubberizing and that production of unrubberized fabrics, including the treated cotton, is also included within the broad scope of the invention.

The temperature at which the treatment with the amine is conducted may vary over wide limits but preferably is between 25° C. and 100° C. In general, the use of temperatures in the upper portion of this range gives better results than temperatures in the lower portion.

The time of treatment may similarly vary widely but preferably ranges from 2 to 60 seconds.

The following reports experimental work which was conducted in accordance with the present invention.

#### Treatment without stretching

In the following data grey cotton cord was treated with aqueous solutions of water-soluble salts of amines of the present invention without stretching. The tensile strength of the cotton cord was measured at 70° F. and 60% relative humidity as is standard in the art. In the tables the expression "RAD" designates the commercially available mixture of disproportionated rosin amines known as "Rosin Amine D" described in the Borglin article mentioned above and comprising as major components dehydroabietylamine, tetrahydroabietylamine, dihydroabietylamine and dextropimarylamine. The treatment, except where otherwise indicated, involved soaking the grey cotton with the aqueous solution of the amine salts for one minute at 95-100° C., followed by vacuum removal of surplus solution and drying at 110° C. In all cases the grey cotton treated was in the form of cord of carded American cotton having the construction known in the art as 12/4/2, a tensile strength of 16.6 pounds when untreated, an elongation at 10 pounds tension of 7.75%, containing 1145 yards per pound and having a gauge of 0.0317 inch. The solutions of the amine salts employed had a pH of 7-8 and contained the indicated percentage of the amine itself rather than the salt thereof.

In the first series of tests the grey cotton cord just described was treated in the manner described with 10% aqueous solutions of RAD formate, acetate, propionate, glycolate, lactate and hydrochloride and of o-aminodicyclohexyl acetate solution. The tensile strengths and ratings of the control and of the treated cords are given in Tables 1 and 2.

Table 1.—RAD salts

#### 10% SOLUTIONS

| Salt               | Tensile |       |
|--------------------|---------|-------|
|                    | Lbs.    | Rtg.  |
| Control.....       | 16.60   | 100.0 |
| Formate.....       | 19.82   | 119.3 |
| Acetate.....       | 19.68   | 118.3 |
| Propionate.....    | 19.16   | 115.3 |
| Glycolate.....     | 19.96   | 120.1 |
| Lactate.....       | 20.19   | 121.4 |
| Hydrochloride..... | 20.33   | 122.5 |

Table 2.—o-Aminodicyclohexyl

#### ACETATE 10% SOLUTION

| 5            | Tensile |       |
|--------------|---------|-------|
|              | Lbs.    | Rtg.  |
| Control..... | 16.60   | 100.0 |
| Acetate..... | 18.58   | 112.0 |

Similar tests reported in Tables 3 and 4 were conducted on the same cotton cord which had been dewaxed by hot alcohol extraction and upon viscose rayon cord, respectively. The results show that no improvement was effected in the dewaxed cotton or rayon by the treatment of the present invention. The rayon cord used was that known in the art as 1650 denier 2 ply.

Table 3.—RAD acetate (10%)

#### EFFECT ON DEWAXED COTTON

| 25               | Tensile |       |
|------------------|---------|-------|
|                  | Lbs.    | Rtg.  |
| Control.....     | 16.60   | 100.0 |
| Dewaxed.....     | 20.65   | 125.0 |
| Dewaxed.....     | 20.65   | 100.0 |
| RAD Acetate..... | 20.73   | 100.3 |

Table 4.—RAD acetate (10%)

#### EFFECT ON RAYON

| 40               | Tensile |       |
|------------------|---------|-------|
|                  | Lbs.    | Rtg.  |
| Control.....     | 22.60   | 100.0 |
| RAD Acetate..... | 20.80   | 92.1  |

Table 5 shows the variation in the activity of several amine salts reported upon in Table 1 as a function of concentration of amine in the aqueous treating solution. In these tests the grey cotton cord described above was used.

Table 5.—RAD salts

#### CONCENTRATION vs. TENSILE

| 55           | RAD    | Formate |       | Acetate |       | Lactate |       | Hydrochloride |      |
|--------------|--------|---------|-------|---------|-------|---------|-------|---------------|------|
|              |        | Tensile |       | Tensile |       | Tensile |       | Tensile       |      |
|              | Conc'n | Lbs.    | Rtg.  | Lbs.    | Rtg.  | Lbs.    | Rtg.  | Lbs.          | Rtg. |
| Control..... | 16.60  | 100.0   | 16.60 | 100.0   | 16.60 | 100.0   | 16.60 | 100.0         |      |
| 2.5%.....    | 19.41  | 117.0   | 18.87 | 113.7   | 19.05 | 114.8   | 18.94 | 114.1         |      |
| 5.0%.....    | 19.70  | 118.7   | 19.52 | 117.5   | 19.82 | 119.5   | 19.29 | 116.2         |      |
| 10.0%.....   | 19.82  | 119.3   | 19.68 | 118.3   | 20.19 | 121.4   | 20.33 | 122.5         |      |
| 20.0%.....   | 19.78  | 119.3   | 20.58 | 123.8   | 20.55 | 123.8   | 20.80 | 125.3         |      |

Grey cotton cord, such as was used in the previous tests, was treated with RAD acetate in the manner described above and was then washed for 10 seconds in tap water at 18° C. The results, reported in Table 6, show that the effect of the treatment with the amine salt is not removed by washing with water.

Table 6.—RAD acetate (10%)  
EFFECT OF WASHING WITH WATER

|                  | Tensile |       |
|------------------|---------|-------|
|                  | Lbs.    | Rtg.  |
| Control          | 16.60   | 100.0 |
| Acetate          | 19.68   | 118.3 |
| Acetate          | 19.68   | 100.0 |
| Acetate and Wash | 19.60   | 99.7  |

The results which are reported in Tables 7 and 8 show that the treatment of the present invention may be satisfactorily conducted over a temperature range of from 25° C. to 100° C. and over a period of time ranging from 2 to 60 seconds.

Table 7.—RAD acetate (10%)  
EFFECT OF TREATING TEMP.

|         | Temp.,<br>°C. | Tensile |       |
|---------|---------------|---------|-------|
|         |               | Lbs.    | Rtg.  |
| Control |               | 16.60   | 100.0 |
| Treat   | 25            | 19.31   | 116.2 |
| Treat   | 100           | 19.68   | 118.3 |

Table 8.—RAD acetate (10%)  
EFFECT OF TREATING TIME

|         | Time,<br>Sec. | Tensile |       |
|---------|---------------|---------|-------|
|         |               | Lbs.    | Rtg.  |
| Control |               | 16.60   | 100.0 |
| Treat   | 2             | 19.30   | 116.2 |
| Treat   | 30            | 19.57   | 117.9 |
| Treat   | 60            | 19.68   | 118.3 |

Grey cotton cord of the above type was treated with RAD acetate as described in connection with Table 1 and was then, without drying, treated at a temperature of 25° C. with a GR-S latex containing 30% solids. The results reported in Table 9 show that the latex treatment does not impair the improvement in tensile strength brought about by the present invention.

Table 9.—RAD acetate (10%)  
EFFECT OF LATEX

|                   | Tensile |       |
|-------------------|---------|-------|
|                   | Lbs.    | Rtg.  |
| Control           | 16.60   | 100.0 |
| Acetate           | 19.68   | 118.3 |
| Acetate           | 19.68   | 100.0 |
| Acetate and Latex | 19.64   | 99.9  |

The chemically treated cord or yarn may be used either in the unstretched condition after treatment with the amine or it may be stretched while wet with the treating solution, or if the treated cotton has been meanwhile dried, it can be rewetted and then stretched with any desired degree of tension. Preferably, the tension imparted to the cords or yarns should be just short

of their breaking point. After the cord or yarn is stretched to the proper extend, it is dried while its stretched length is maintained, that is, without permitting shrinkage, and as referred to in British Patent No. 545,716 involving drying while maintaining the cord or yarn under a uniform state of length.

#### TREATMENT WITH STRETCHING

10 The following experimental work illustrates the practice of my invention wherein grey cotton yarn which had been treated with a solution of the amine was stretched or tensioned to a point just short of its breaking point while still wet with the treating solution and was then dried under the resulting tension.

15 The grey cotton yarn used was that known in the art as 6.60/6 Karnak. In the first series of tensioning tests the yarn was soaked for approximately one minute with a 1.75% aqueous solution of "Rosin Amine D" acetate (containing 1.75% by weight of the amine), was tensioned while wet to a point just short of its breaking point and was then dried under the resulting tension at 20 110° C. The tensile strength of the resulting yarn was 39.43 pounds in comparison to a tensile strength of 25.99 pounds for the untreated yarn or an improvement of 51.7%.

25 In another series of experiments the same grey cotton yarn was treated in exactly same manner with an aqueous solution consisting of 70% by volume of a 1.75% by weight solution of sodium abietate and 30% by volume of a 1.75% by weight solution of "Rosin Amine D" acetate. The resulting yarn had a tensile strength of 40.22 pounds compared to 25.11 pounds for the untreated yarn or an improvement of 60.2%. With a 1.75% solution of sodium abietate alone, the treated yarn had a tensile strength of 39.62 pounds or an improvement of 57.8% over the control. This illustrates that an unexpected increase in tensile strength is made possible by using the amines of the present invention in combination with alkali metal salts of rosin acids, since the increase obtained with the combination is greater than the increase obtained with either the amine alone or the alkali metal salt of the rosin acid alone. The relative proportions 30 of the amine and the alkali salt of the rosin acid may vary widely, say from 20% up to 100% of the amine and correspondingly from 80% to 0% of the alkali metal salt of the rosin acid.

40 In still another series of experiments the same grey cotton yarn was first treated with a 10% aqueous solution of trisodium phosphate, dried, then soaked as before in the same 1.75% solution of "Rosin Amine D" acetate, tensioned as before while wet therewith and then dried under the resulting tension. The tensile strength of the resulting yarn was 40.86 pounds in comparison to a tensile strength of 25.11 pounds for the control. This shows that precipitation of the rosin amine 45 as the insoluble rosin amine phosphate gives results equivalent to those obtained where the amine is present in the treated cotton in the form of a water-soluble salt thereof.

50 A very important advantage of the treatment of the present invention is that it adds greatly to the mildew-resistance of the yarn or cord. Thus, the same grey cotton yarn that was used in the preceding tests was exposed to mildew fungi for a period of four weeks at room temperature 55 and 100% relative humidity. Samples of both

untreated yarn and yarn which had been treated with the 1.75% solution of "Rosin Amine D" acetate, followed by tensioning and drying as in the preceding tests, were exposed to these mildewing conditions. At the end of the tests, the treated yarn had a tensile strength of 34.09 pounds in comparison to a strength of 39.43 pounds at the beginning of the tests, whereas the untreated yarn had a tensile strength of 15.30 pounds after exposure in comparison to a strength of 26.79 pounds at the beginning of exposure. Thus, the treated yarn had considerably more strength after exposure than the untreated yarn had before exposure. The percentage reduction in strength as a result of the mildewing exposure was 42.8% for the untreated yarn as against only 13.6% for the treated yarn.

While the foregoing description is chiefly concerned with improving the tensile strength of grey cotton fibers, it may be extended to naturally occurring cellulosic fibers in general which have substantially their native composition, for example, flax, hemp, jute, etc.

Having thus described my invention, what I claim and desire to protect by Letters Patent is:

1. Grey cotton containing at least 75% of the original naturally occurring waxes and having an improved tensile strength as a result of impregnation with dehydroabietylamine in an inert liquid medium.

2. Grey cotton containing at least 75% of the original naturally occurring waxes and having an improved tensile strength as a result of impregnation with dihydroabietylamine in an inert liquid medium.

3. Grey cotton containing at least 75% of the original naturally occurring waxes and having an improved tensile strength as a result of impregnation with tetrahydroabietylamine in an inert liquid medium.

4. Grey cotton containing at least 75% of the original naturally occurring waxes and having an improved tensile strength as a result of impregnation with a mixture comprising dehydroabietylamine, dihydroabietylamine, tetrahydroabietylamine and dextropimarylamine in an inert liquid medium.

5. Grey cotton containing at least 75% of the original naturally occurring waxes and having an improved tensile strength as a result of impregnation with an aqueous solution of a mixture of water-soluble salts of dehydroabietylamine, dihydroabietylamine, tetrahydroabietylamine and dextropimarylamine.

6. Naturally occurring cellulosic fibers containing at least 75% of the original naturally occurring waxes and having an improved tensile strength as a result of impregnation with a mixture of primary rosin amines comprising dehydroabietylamine, dihydroabietylamine, tetrahydroabietylamine and dextropimarylamine and sodium abietate in an inert liquid medium.

7. Naturally occurring cellulosic fibers containing at least 75% of the original naturally occurring waxes and having an improved tensile strength as a result of impregnation with an aqueous solution comprising water-soluble salts of dehydroabietylamine, dihydroabietylamine, tetrahydroabietylamine and dextropimarylamine and sodium abietate.

8. A process of improving the tensile strength of naturally occurring cellulosic fibers containing at least 75% of the original naturally occurring waxes which comprises impregnating said fibers with a compound selected from the group

consisting of primary rosin amines having the general formula



where ring A is hydroaromatic, ring B is a ring selected from the group consisting of hydroaromatic and semi-aromatic rings, ring C is a ring selected from the group consisting of hydroaromatic, semi-aromatic and aromatic rings, and R is selected from the group consisting of



and water-soluble salts of said amines, said compound being applied in an inert liquid medium.

9. A process of improving the tensile strength of grey cotton containing at least 75% of the original naturally occurring waxes and which comprises impregnating said grey cotton with a compound selected from the group consisting of primary rosin amines having the general formula



where ring A is hydroaromatic, ring B is a ring selected from the group consisting of hydroaromatic and semi-aromatic rings, ring C is a ring selected from the group consisting of hydroaromatic, semi-aromatic and aromatic rings, and R is selected from the group consisting of



and water-soluble salts of said amines, said compound being applied in an inert liquid medium.

10. A process of improving the tensile strength of grey cotton containing at least 75% of the original naturally occurring waxes and which comprises impregnating said grey cotton with an aqueous solution of a water-soluble salt of a primary rosin amine having the general formula



where ring A is hydroaromatic, ring B is a ring selected from the group consisting of hydroaromatic and semi-aromatic rings, ring C is a ring selected from the group consisting of hydro-

11

aromatic, semi-aromatic and aromatic rings, and R is selected from the group consisting of



11. A process as in claim 10 wherein the concentration of said amine in said solution is from 0.5% to 20%, said percentages being by weight.

12. A process as in claim 10 wherein the concentration of said amine in said solution is from 0.5% to 20%, said percentages being by weight, and wherein said impregnating is carried on at a temperature of from 25° C. to 100° C. and for a time of from 2 to 60 seconds.

13. Naturally occurring cellulosic fibers containing at least 75% of the original naturally occurring waxes and having an improved tensile strength as a result of impregnation with a compound selected from the group consisting of primary rosin amines having the general formula



where ring A is hydroaromatic, ring B is a ring selected from the group consisting of hydroaromatic and semi-aromatic rings, ring C is a ring selected from the group consisting of hydroaromatic, semi-aromatic and aromatic rings, and R is selected from the group consisting of



and water-soluble salts of said amines, said compounds being applied in an inert liquid medium.

14. Grey cotton containing at least 75% of the original naturally occurring waxes and having an improved tensile strength as a result of impregnation with a compound selected from the group consisting of primary rosin amines having the general formula



12

where ring A is hydroaromatic, ring B is a ring selected from the group consisting of hydroaromatic and semi-aromatic rings, ring C is a ring selected from the group consisting of hydroaromatic, semi-aromatic and aromatic rings, and R is selected from the group consisting of



and water-soluble salts of said amines, said compound being applied in an inert liquid.

15. Grey cotton containing at least 75% of the original naturally occurring waxes and having an improved tensile strength as a result of impregnation with an aqueous solution of a water-soluble salt of a primary rosin amine having the general formula



where ring A is hydroaromatic, ring B is a ring selected from the group consisting of hydroaromatic and semi-aromatic rings, ring C is a ring selected from the group consisting of hydroaromatic, semi-aromatic and aromatic rings, and R is selected from the group consisting of



JOSEPH M. ALMAND.

#### REFERENCES CITED

The following references are of record in the file of this patent:

#### UNITED STATES PATENTS

| Number    | Name             | Date           |
|-----------|------------------|----------------|
| 2,186,101 | Dreyfus          | Jan. 9, 1940   |
| 2,194,429 | Krzikalla et al. | Mar. 19, 1940  |
| 2,201,237 | Littmann         | May 21, 1940   |
| 2,297,536 | Buckwalter       | Sept. 29, 1942 |
| 2,423,469 | Schlosser et al. | July 8, 1947   |

55